



US010763068B2

(12) **United States Patent**  
**Hayashi et al.**

(10) **Patent No.:** **US 10,763,068 B2**  
(45) **Date of Patent:** **Sep. 1, 2020**

(54) **ELECTRON EMISSION ELEMENT AND METHOD FOR SAME**

(71) Applicant: **Sharp Kabushiki Kaisha**, Sakai, Osaka (JP)

(72) Inventors: **Hidekazu Hayashi**, Sakai (JP); **Tokio Taguchi**, Sakai (JP); **Kenichiro Nakamatsu**, Sakai (JP); **Tadashi Iwamatsu**, Sakai (JP); **Kohji Shinkawa**, Sakai (JP); **Mai Takasaki**, Sakai (JP); **Toshihiro Kaneko**, Sakai (JP); **Atsushi Niinoh**, Sakai (JP)

(73) Assignee: **SHARP KABUSHIKI KAISHA**, Sakai (JP)

(\*) Notice: Subject to any disclaimer, the term of this patent is extended or adjusted under 35 U.S.C. 154(b) by 0 days.

(21) Appl. No.: **16/613,540**

(22) PCT Filed: **May 15, 2018**

(86) PCT No.: **PCT/JP2018/018713**

§ 371 (c)(1),  
(2) Date: **Nov. 14, 2019**

(87) PCT Pub. No.: **WO2018/212166**

PCT Pub. Date: **Nov. 22, 2018**

(65) **Prior Publication Data**

US 2020/0075285 A1 Mar. 5, 2020

(30) **Foreign Application Priority Data**

May 18, 2017 (JP) ..... 2017-098997  
Jun. 19, 2017 (JP) ..... 2017-119726

(51) **Int. Cl.**

**H01J 1/312** (2006.01)

**H01J 9/02** (2006.01)

**H01J 9/42** (2006.01)

(52) **U.S. Cl.**

CPC ..... **H01J 1/312** (2013.01); **H01J 9/022** (2013.01); **H01J 9/42** (2013.01)

(58) **Field of Classification Search**

CPC ..... H01J 1/312; H01J 9/022; H01J 9/42

See application file for complete search history.

(56) **References Cited**

U.S. PATENT DOCUMENTS

2006/0138664 A1 6/2006 Ito et al.  
2010/0278561 A1 11/2010 Kanda et al.

FOREIGN PATENT DOCUMENTS

JP 2001-143600 A 5/2001  
JP 2003-229045 A 8/2003

(Continued)

OTHER PUBLICATIONS

English translation of JP 2004-014406 (Year: 2004).\*

(Continued)

Primary Examiner — Anne M Hines

(74) Attorney, Agent, or Firm — Keating & Bennett, LLP

(57) **ABSTRACT**

An electron emitting device (100) includes a first electrode (12), a second electrode (52), and a semi-conductive layer (30) provided between the first electrode (12) and the second electrode (52). The semi-conductive layer (30) includes a porous alumina layer (32) having a plurality of pores (34) and silver (42) supported in the plurality of pores (34) of the porous alumina layer (32).

**13 Claims, 8 Drawing Sheets**



(56)

**References Cited**

FOREIGN PATENT DOCUMENTS

|    |               |        |
|----|---------------|--------|
| JP | 2004-014406 A | 1/2004 |
| JP | 2004-178863 A | 6/2004 |
| JP | 2009-146891 A | 7/2009 |
| JP | 2016-136485 A | 7/2016 |

OTHER PUBLICATIONS

Iwamatsu et al., "Novel Charging System by Electron Emission Device in the Atmosphere", Journal of the Imaging Society of Japan, vol. 56, No. 1, 2017, 5 pages.

Nakamatsu et al., "Electron Emission Device, Method for Manufacturing Same, and Method for Manufacturing Electronic Device", U.S. Appl. No. 16/127,670, filed Sep. 11, 2018.

Nakamatsu et al., "Electron Emission Device and Method for Manufacturing the Same", U.S. Appl. No. 16/369,004, filed Mar. 29, 2019.

Official Communication issued in International Patent Application No. PCT/JP2018/018713, dated Aug. 14, 2018.

\* cited by examiner

*FIG. 1**FIG. 2*

(a)



(b)



(c)



FIG.3



FIG. 4

(a)



(b)



(c)



FIG.5

(a)



1 μm

(b)



500nm

*FIG. 6*

(a)



(b)



(c)



FIG. 7



FIG. 8



FIG.9



FIG.10



FIG.11



FIG.12



## 1

ELECTRON EMISSION ELEMENT AND  
METHOD FOR SAME

## TECHNICAL FIELD

The present invention relates to an electron emitting device and a method of producing the same.

## BACKGROUND ART

The applicant has developed electron emitting devices having a novel structure, which are capable of operating in the atmospheric air (see, for example, Patent Documents 1 and 2).

The electron emitting device which is described in Patent Document 2 includes a semi-conductive layer which is interposed between a pair of electrodes (i.e., a substrate electrode and a surface electrode), the semi-conductive layer being composed of a dielectric material with electrically conductive nanoparticles dispersed therein. By applying a voltage on the order of several dozen volts to the semi-conductive layer, electrons can be emitted from the surface electrode (field electron emission). Therefore, unlike any conventional electron emitting device (e.g., a corona discharger) that utilizes a discharge phenomenon under a strong field, this electron emitting device has an advantage in that ozone will not be generated.

This electron emitting device can be suitably used as a charger device for charging a photosensitive drum of an image forming apparatus (e.g., a copier machine), for example. According to Non-Patent Document 1, an electron emitting device that includes a surface electrode of the layered structure described in Patent Document 2 may have a lifetime of about 300 hours (equivalent to approximately 300,000 sheets in the case of a medium-fast copier machine) or more.

## CITATION LIST

## Patent Literature

[Patent Document 1] Japanese Laid-Open Patent Publication No. 2009-146891 (Japanese Patent No. 4303308)

[Patent Document 2] Japanese Laid-Open Patent Publication No. 2016-136485

## Non-Patent Literature

[Non-Patent Document 1] Tadashi IWAMATSU et al., NIHON GAZO GAKKAISHI (Journal of the Imaging Society of Japan), Vol. 56, No. 1, pp. 16-23, (2017)

## SUMMARY OF INVENTION

## Technical Problem

However, there is a desire to improve the characteristics and/or prolong the lifetime of the aforementioned electron emitting device. Accordingly, an objective of the present invention is to provide: an electron emitting device having a novel structure, such that the characteristics of the electron emitting device can be improved and/or its lifetime can be prolonged; and a method of producing the same.

## Solution to Problem

An electron emitting device according to an embodiment of the present invention comprises a first electrode, a second

## 2

electrode, and a semi-conductive layer provided between the first electrode and the second electrode, wherein the semi-conductive layer includes a porous alumina layer having a plurality of pores and silver supported in the plurality of pores of the porous alumina layer.

In one embodiment, the first electrode is formed of an aluminum substrate or an aluminum layer, and the porous alumina layer is an anodized layer formed at a surface of the aluminum substrate or at a surface of the aluminum layer.

10 In one embodiment, the first electrode is formed of an aluminum substrate containing aluminum in an amount of not less than 99.00 mass % but less than 99.99 mass %, and the porous alumina layer is an anodized layer formed at a surface of the aluminum substrate.

15 In one embodiment, aluminum is contained in an amount of 99.98 mass % or less in the aluminum substrate.

In one embodiment, the porous alumina layer has a thickness which is not less than 10 nm and not more than 5  $\mu$ m.

20 In one embodiment, the plurality of pores have an opening having a two-dimensional size which is not less than 50 nm and not more than 3  $\mu$ m as viewed from a normal direction of a surface thereof.

In one embodiment, the plurality of pores of the porous alumina layer have a depth which is not less than 10 nm and not more than 5  $\mu$ m. The plurality of pores of the porous alumina layer may have a depth which is not less than 50 nm and not more than 500 nm.

In one embodiment, a barrier layer included in the porous alumina layer has a thickness which is not less than 1 nm and not more than 1  $\mu$ m. A barrier layer included in the porous alumina layer may have a thickness of 100 nm or less.

25 In one embodiment, the plurality of pores of the porous alumina layer have a stepped side surface. The plurality of pores have, along a depth direction, two or more pore subportions with mutually differing pore diameters, such that any pore subportion at a deeper position has a smaller pore diameter.

In one embodiment, the silver contains silver nanoparticles having an average particle size which is not less than 1 nm and not more than 50 nm. The silver may contain silver nanoparticles with an average particle size which is not less than 3 nm and not more than 10 nm.

30 In one embodiment, the second electrode includes a gold layer. The second electrode has the layered structure described in Patent Document 2.

A method of producing an electron emitting device according to an embodiment of the present invention is a method of producing any of the above electron emitting devices, comprising: a step of providing an aluminum substrate or an aluminum layer supported by a substrate; a step of anodizing a surface of the aluminum substrate or the aluminum layer to form a porous alumina layer; and a step of applying silver nanoparticles in a plurality of pores of the porous alumina layer.

In one embodiment, the step of forming the porous alumina layer comprises an anodization step and an etching step to be performed after the anodization step.

35 In one embodiment, the step of forming the porous alumina layer comprises a further anodization step after the etching step.

## Advantageous Effects of Invention

65 According to an embodiment of the present invention, there is provided: an electron emitting device having an a novel structure such that its characteristics can be improved

and/or its lifetime can be prolonged as compared to the aforementioned conventional technique; and a method of producing the same.

#### BRIEF DESCRIPTION OF DRAWINGS

FIG. 1 A schematic cross-sectional view of an electron emitting device 100 according to an embodiment of the present invention.

FIG. 2 (a) through (c) are schematic cross-sectional views for describing a method of producing the electron emitting device 100 according to an embodiment of the present invention.

FIG. 3 (a) through (c) are schematic cross-sectional views showing examples of porous alumina layers for use as the semi-conductive layer of the electron emitting device 100.

FIG. 4 (a) through (c) are schematic cross-sectional views showing differing states of silver nanoparticles in a semi-conductive layer 30A, in an electron emitting device according to an embodiment of the present invention.

FIGS. 5 (a) and (b) are diagrams showing cross-sectional STEM images of a semi-conductive layer containing silver nanoparticles.

FIG. 6 (a) through (c) are diagrams showing results of EDX analysis in a cross section (inside open circles 6a, 6b and 6c in FIG. 5(b)) of a semi-conductive layer.

FIG. 7 A diagram schematically showing a measurement system for the electron emission characteristics of the electron emitting device 100.

FIG. 8 A diagram showing a result of an energization test for an electron emitting device according to Example.

FIG. 9 A schematic cross-sectional view showing an electron emitting device 200 according to Comparative Example.

FIG. 10 A diagram showing a result of an energization test for the electron emitting device of Comparative Example.

FIG. 11 A diagram showing a cross-sectional STEM image of a semi-conductive layer containing silver nanoparticles, in the electron emitting device of Comparative Example.

FIG. 12 A diagram showing a result of EDX analysis in a cross section (a region indicated with an open circle 2a in FIG. 11) of the semi-conductive layer of the electron emitting device of Comparative Example.

#### DESCRIPTION OF EMBODIMENTS

Hereinafter, with reference to the drawings, electron emitting devices according to embodiments of the present invention and methods of producing the same will be described. Embodiments of the present invention are not to be limited to the illustrated embodiments. In the following description, constituent elements with like functions are denoted by like reference numerals, and redundant description will be avoided.

FIG. 1 shows a schematic cross-sectional view of an electron emitting device 100 according to an embodiment of the present invention.

The electron emitting device 100 includes a first electrode 12, a second electrode 52, and a semi-conductive layer 30 provided between the first electrode 12 and the second electrode 52. The first electrode 12 is composed of an aluminum substrate 12 (e.g., a thickness of 0.5 mm), for example, whereas the second electrode 52 is composed of a gold (Au) layer (e.g., 40 nm thick), for example. The dielectric layer 22 may function as a device separation layer when a plurality of electron emitting devices 100 are to be

produced on an aluminum substrate. The size of a single electron emitting device 100 (i.e., the size of a region surrounded by the dielectric layer 22) may be e.g., about 5 mm×about 5 mm (5 mm<sup>2</sup>), and the dielectric layer 22 has a width of about 5 mm. The dielectric layer 22 may be omitted when just forming a single electron emitting device 100. However, providing the dielectric layer 22 may result in the advantages of an ability to restrain a concentrated electric field and a leakage current from occurring between the first electrode 12 and the second electrode 52.

The semi-conductive layer 30 includes a porous alumina layer 32 having a plurality of pores 34 and silver (Ag) 42 that is supported in the plurality of pores 34 of the porous alumina layer 32.

The plurality of pores 34 have an opening whose two-dimensional size (Dp) as viewed from the normal direction of its surface is not less than about 50 nm and not more than about 3  $\mu$ m, for example. The plurality of pores 34 may have an opening whose two-dimensional size (Dp) as viewed from the normal direction of its surface is less than about 500 nm. In the present specification, an “opening” refers to an uppermost portion of a pore 34. If a pore 34 has two or more pore subportions with mutually differing pore diameters along the depth direction, regarding the pore diameter, the pore diameter of the uppermost portion is referred to as the opening diameter. The “two-dimensional size” means an area equivalent circle diameter of the opening (pore 34) as viewed from the normal direction of its surface. In the following description, any reference to “two-dimensional size”, “opening diameter”, or “pore diameter” is intended to be an area equivalent circle diameter. Details of the porous alumina layer 32 will be described later with reference to FIG. 3.

The silver supported in the pores 34 may be, for example, nanoparticles of silver (hereinafter denoted as “Ag nanoparticles”). The Ag nanoparticles preferably have an average particle size of not less than 1 nm and not more than 50 nm, for example. More preferably, the Ag nanoparticles have an average particle size of not less than 3 nm and not more than 10 nm, for example. The Ag nanoparticles may be coated with an organic compound (e.g., an alcohol derivative and/or surfactant).

The first electrode 12 is composed of an aluminum substrate (e.g., 0.5 mm thick), for example, whereas the porous alumina layer 32 is an anodized layer formed on the surface of the aluminum substrate. Instead of an aluminum substrate, an aluminum layer which is formed on a substrate (e.g., a glass substrate) may be used. In other words, the porous alumina layer 32 may be an anodized layer which is formed at the surface of an aluminum layer that is supported by a substrate. In this case, if the substrate is a dielectric substrate such as a glass substrate, an electrically conductive layer may be formed between the aluminum layer and the substrate, and the aluminum layer and the electrically conductive layer may be utilized as electrodes. Any aluminum layer (i.e., a portion remaining after anodization) functioning as an electrode preferably has a thickness of e.g. 10  $\mu$ m or more.

The second electrode 52 is composed of a gold (Au) layer, for example. The Au layer preferably has a thickness of not less than 10 nm and not more than 100 nm, e.g. 40 nm. Otherwise, platinum (Pt) may be used. Furthermore, as described in Patent Document 2, a layered structure of an Au layer and a Pt layer may be adopted; in this case, preferably the Au layer serves as a lower layer and the Pt layer serves as an upper layer in the layered structure (Pt layer/Au layer). In the layered structure, the Pt layer preferably has a

thickness of not less than 10 nm and not more than 100 nm, e.g. 20 nm, and the Au layer preferably has a thickness of not less than 10 nm and not more than 100 nm, e.g. 20 nm. As compared to forming the second electrode 52 with an Au layer alone, the Pt layer/Au layer layered structure can provide a lifetime which is about 5 times longer.

Next, with reference to FIG. 2, a method of producing the electron emitting device 100 will be described. FIGS. 2(a) through (c) show schematic cross-sectional views for describing a method of producing the electron emitting device 100 according to an embodiment of the present invention.

First, as shown in FIG. 2(a), an aluminum substrate 12 having a dielectric layer 22 partially formed therein is provided. As the aluminum substrate 12, for example, JIS A1050 (thickness: 0.5 mm) may be used. The dielectric layer 22 may be formed by performing an anodization (alumite treatment) and a sealing treatment while masking a device formation region of the surface of the aluminum substrate 12, for example. The dielectric layer 22 is formed by performing an anodization with sulfuric acid (15 wt %, 20° C.±1° C.) for 250 seconds to 300 seconds at a current density of 1 A/dm<sup>2</sup> to form a porous alumina layer with a thickness of 2 μm to 4 μm, and thereafter performing a sealing treatment for the porous alumina layer with distilled water (pH: 5.5 to 7.5, 90° C.) for about 30 minutes, for example.

As necessary, the surface of the aluminum substrate may be subjected to a pretreatment. For example, a microblasting treatment may be performed. Alternatively, after a porous alumina layer is formed through anodization, the porous alumina layer may be removed by etching. The pores in the porous alumina layer to be first formed are likely to be distributed irregularly (randomly). Therefore, in order to form a porous alumina layer with a regular array of pores, it is preferable to remove the porous alumina layer that was formed first.

Next, as shown in FIG. 2(b), the surface of the aluminum substrate 12 is anodized in order to form the porous alumina layer 32. As will be described later with reference to FIG. 3, the anodization may be followed by an etching as necessary. Anodization and etching may be alternated a plurality of times. By adjusting the conditions of anodization and etching, pores 34 with various cross-sectional shapes and sizes can be formed.

Next, as shown in FIG. 2(c), silver (Ag) 42 is allowed to be supported in the pores 34 of the porous alumina layer 32. In the case where Ag nanoparticles are used as Ag, a dispersion obtained by dispersing Ag nanoparticles in an organic solvent (e.g., toluene) is applied onto the porous alumina layer 32. The Ag nanoparticles within the dispersion may be coated with an organic compound (e.g., an alcohol derivative and/or a surfactant). The content ratio of Ag nanoparticles in the dispersion is preferably e.g. not less than 0.1 mass % and not more than 10 mass %, and may be 2 mass %, for example. The method of applying the dispersion is not particularly limited. For example, spin coating, spray coating, or the like may be used.

Next, with reference to FIG. 3, the structure of the porous alumina layer 32 of the electron emitting device 100 will be described. The porous alumina layer 32 may be any of porous alumina layers 32A, 32B and 32C shown in FIGS. 3(a), (b) and (c), for example. Moreover, without being limited to the porous alumina layers 32A, 32B and 32C, the porous alumina layer 32 admits of various modifications, as will be described below.

The porous alumina layer is formed by, for example, allowing the surface of an aluminum substrate (within which

portions that were not anodically oxidized will become the first electrode 12) to undergo anodization in an acidic electrolytic solution. The electrolytic solution to be used in the step of forming the porous alumina layer may be, for example, an aqueous solution that contains an acid which is selected from the group consisting of oxalic acid, tartaric acid, phosphoric acid, chromic acid, citric acid, and malic acid. By adjusting the conditions of anodization (e.g., the kind of electrolytic solution, applied voltage), it is possible to control the opening diameter Dp, the interpore distance Dint, the pore depth Dd, the thickness tp of the porous alumina layer, and the thickness tb of the barrier layer. A porous alumina layer which is obtained through anodization may have, for example, cylindrical pores 34B as in the porous alumina layer 32B shown in FIG. 3(b).

After the anodization, the porous alumina layer may be placed in contact with an etchant for alumina and subjected to a predetermined amount of etching so as to enlarge the pore diameter. With wet etching, the pore wall and the barrier layer can be etched substantially isotropically. By adjusting the kind of etchant and its concentration, as well as the etching time, it is possible to control the etching amount (that is, the opening diameter Dp, interpore distance Dint, pore depth Dd, the barrier layer thickness tb, etc.). Examples of etchants that may be used are: an aqueous solution of phosphoric acid; an aqueous solution of an organic acid, e.g., formic acid, acetic acid, or citric acid; or a chromic and phosphoric acid mixture aqueous solution. A porous alumina layer which is obtained by performing etching only once after the anodization will have cylindrical pores 34B, as in the porous alumina layer 32B illustrated in FIG. 3(b). However, the opening diameter Dp of the pores 34B and the thickness tb of the barrier layer 32b have changed through the etching.

For example, an anodization may be performed with oxalic acid (0.05 M, 5° C.) and a formation voltage of 80 V for about 25 minutes; thereafter, 20 minutes of etching may be performed with phosphoric acid (0.1 M, 25° C.); as a result, a porous alumina layer 32B having a depth Dd of about 2000 nm, an opening diameter Dp of 100 nm, an interpore distance Dint of 200 nm, and a barrier layer thickness tb of about 30 nm can be obtained.

In another example, for example, an anodization may be performed with oxalic acid (0.05 M, 5° C.) and a formation voltage of 80 V for about 10 minutes; thereafter, 20 minutes of etching may be performed with phosphoric acid (0.1 M, 25° C.); as a result, a porous alumina layer 32B having a depth Dd of about 700 nm, an opening diameter Dp of 100 nm, an interpore distance Dint of 200 nm, and a barrier layer thickness tb of 50 nm can be obtained.

After the etching step, a further anodization may be performed to grow the pores in the depth direction, and also to thicken the porous alumina layer. Since the pore growth begins from the bottoms of the pores that have already been formed, each pore will have a stepped side surface. As a result, pores 34A having a stepped side surface are obtained, as in the pores 34A illustrated in FIG. 3(a). Along the depth direction, each pore 34A has two pore subportions with mutually differing pore diameters, such that the pore subportion at a deeper position has a smaller pore diameter. For example, as shown in FIG. 3(a), the subportion at a deeper position (depth Dd1, pore diameter Dp1) has a smaller pore diameter Dp1 than the opening diameter Dp. A pore 34A having a stepped side surface is capable of catching an Ag nanoparticle(s) at the step portion(s), thus providing an advantage of being able to support many Ag nanoparticles in the pore 34A. For example, among the plurality of pores 34,

any pore that has an opening diameter which is not less than about 100 nm and not more than about 3  $\mu\text{m}$  preferably includes a pore subportion at a deeper position, this pore subportion having a pore diameter of not less than 50 nm and not more than 500 nm.

The porous alumina layer 32A may be formed in the following manner, for example. An anodization may be performed with oxalic acid (0.05 M, 5° C.) and a formation voltage of 80 V for about 10 minutes; thereafter, 20 minutes of etching with phosphoric acid (0.1 M, 25° C.) is performed; thereafter again, an anodization may be performed with oxalic acid (0.05 M, 5° C.) and a formation voltage of 80 V for about 20 minutes; as a result, a porous alumina layer 32A having a depth Dd of about 1500 nm, an opening diameter Dp of 100 nm, an interpore distance Dint of 200 nm, and a barrier layer thickness tb of 50 nm can be obtained. Herein, along the depth direction, each pore 34A has two pore subportions with mutually differing pore diameters, such that it has a pore subportion with a depth Dd1 of 500 nm and a pore diameter Dp1 of about 20 nm at a deeper position.

Further thereafter, as necessary, the porous alumina layer may be placed in contact with an etchant for alumina in order to perform further etching, thus further enlarging the pore diameter. As the etchant, the aforementioned etchants are preferable here also.

By repeating anodization steps and etching steps, pores can be formed each having two or more pore subportions with mutually differing pore diameters along the depth direction, such that any pore subportion at a deeper position has a smaller pore diameter, for example. Furthermore, as in the porous alumina layer 32C illustrated in FIG. 3(c), pores 34C each having a sloped side surface (note that sufficiently small steps will result in the appearance of a slope) can be formed. The overall shape of each pore 34C is substantially conical (although the cone is situated upside down). The applicant has established a technique of mass-producing an antireflection film having a moth-eye structure by using a porous alumina layer having conical pores as a mold.

As described above, the porous alumina layer 32 may be any of the porous alumina layers 32A, 32B and 32C shown in FIGS. 3(a), (b) and (c), but admits of various modifications without being limited to these. Regardless of the shape of the porous alumina layer 32, the thickness tp of the porous alumina layer 32 is not less than about 10 nm and not more than about 5  $\mu\text{m}$ , for example. If it is thinner than 10 nm, enough silver (e.g., Ag nanoparticles) cannot be supported, so that a desired electron emission efficiency may be not be obtained. Although there is no upper limit for the thickness tp of the porous alumina layer 32, the electron emission efficiency tends to be saturated even if the porous alumina layer 32 becomes any thicker; thus, from a production efficiency standpoint, there is no need for a thickness that is greater than 5  $\mu\text{m}$ .

The depth Dd of the plurality of pores 34 in the porous alumina layer 32 may be e.g. not less than 10 nm and not more than 5  $\mu\text{m}$ . The depth Dd of the plurality of pores 34 may be e.g. not less than 50 nm and not more than 500 nm. The depth Dd of the plurality of pores 34 may be set as appropriate, depending on the thickness of the porous alumina layer 32.

The thickness tb of the barrier layer 32b of the porous alumina layer 32 is preferably not less than 1 nm and not more than 1  $\mu\text{m}$ . More preferably, the thickness tb of the barrier layer 32b is 100 nm or less. The barrier layer 32b is a layer constituting the bottom of the porous alumina layer 32. If the barrier layer 32b is thinner than 1 nm, short-

circuiting may occur upon voltage application; on the other hand, if it is thicker than 1  $\mu\text{m}$ , a sufficient voltage may not be applied to the semi-conductive layer 30. Generally speaking, the thickness tb of the barrier layer 32b of the porous alumina layer 32 depends on the interpore distance Dint and the opening diameter (two-dimensional size) Dp of the pores 34 and the conditions of anodization.

Hereinafter, by way of experimental examples, the electron emitting device 100 according to an embodiment of the present invention will be described in more detail.

FIGS. 4(a), (b) and (c) are schematic cross-sectional views showing differing states of silver nanoparticles in the semi-conductive layer 30A, in an electron emitting device according to an embodiment of the present invention. FIG. 4(a) shows a state immediately after the semi-conductive layer 30A is formed; FIG. 4(b) shows a state after a “forming” treatment but before being driven; and FIG. 4(c) shows the structure during stable operation. These are all schematic illustrations based on results of observing a cross section of a prototyped device with a scanning transmission electron microscope (hereinafter “STEM”).

The semi-conductive layer 30A is obtained by allowing Ag nanoparticles 42n to be supported in the porous alumina layer 32A which has been formed as described above, for example.

For the Ag nanoparticles, for example, an Ag nanoparticle dispersion obtained by dispersing alcohol derivative-coated Ag nanoparticles in an organic solvent (an average particle size of the alcohol derivative-coated Ag nanoparticles: 6 nm, dispersion solvent: toluene, Ag concentration: 1.3 mass %) can be used. For example, on a porous alumina layer 32A that is formed in a region of about 5 mm  $\times$  about 5 mm, 200  $\mu\text{L}$  (microliters) of the aforementioned Ag nanoparticle dispersion is added dropwise; and spin coating is performed under conditions of: e.g. 500 rpm for 5 seconds and thereafter 1500 rpm for 10 seconds. Thereafter, baking is performed at 150° C. for 1 hour, for example. For enhanced dispersibility, the Ag nanoparticles are coated with an organic substance having e.g. alkoxide and/or carboxylic acid, or a derivative thereof at its terminal end. The baking step is able to remove or reduce the organic substance.

The semi-conductive layer 30A which has just been formed, the Ag nanoparticles 42n abound in lower portions of the pores 34A, as shown in FIG. 4(a).

Once the “forming” treatment is performed, as shown in FIG. 4(b), in some pores 34A, the Ag nanoparticles 42n are arrayed along the depth direction of the pores 34A, thereby being distributed to near the opening of the pore 34A. Electrons will be emitted from any pore 34A (the third pore 34A from the left in FIG. 4(b)) in which the Ag nanoparticles 42n are thus distributed to near the opening. Note that the “forming” treatment refers to a treatment that involves energization for realizing stable electron emission. Although depending on the structure of the semi-conductive layer 30A, the “forming” treatment is performed by, as the voltage to be applied to the electron emitting device 100 (e.g., a driving voltage Vd as shown in FIG. 7), using a rectangular wave having e.g. a frequency of 2 kHz and a duty ratio of 0.5, and increasing this voltage to about 20 V at a rate of 0.1 V/sec. In the present specification, the voltage to be applied to the electron emitting device 100 is expressed in terms of the potential of the second electrode 52 relative to the potential of the first electrode 12. When the voltage to be applied to the electron emitting device 100 is 20 V, for example, the potentials of the first electrode and the second electrode 52 are e.g. -20 V and 0 V, respectively. However, without being limited to this example, the potential of the

first electrode **12** may be the ground potential, and the potential of the second electrode **52** may be a positive value.

While electrons are being stably emitted, as shown in FIG. 4(c), it is considered that pores **34A** in which the Ag nanoparticles **42n** are distributed to near the opening are being consecutively formed.

Thereafter, a phenomenon occurs such that the porous alumina layer **32** is locally destroyed. This is presumably because of heat generation that is caused by electron emission.

FIGS. 5(a) and (b) show example cross-sectional STEM images of the semi-conductive layer (which has not been energized yet) of the prototyped device. FIG. 5(b) shows an enlarged image of the region surrounded by a broken line **5b** in FIG. 5(a). FIGS. 6(a), (b) and (c) show results of energy dispersive X-ray analysis (hereinafter “EDX”) of regions indicated by open circles **6a**, **6b** and **6c** in FIG. 5(b) (i.e., vicinities of dark dots that are considered to be the Ag nanoparticles). DB-Strata237 (available from Japan FEI) was used as the STEM, and Genesis2000 (available from EDAX, Inc.) was used as the EDX. Unless otherwise specified, this will also be the case hereinafter.

As can be seen from FIG. 5(a), pores extend along the normal direction with respect to the surface. Since presence of Ag is confirmed in FIGS. 6(a), (b) and (c), the dark dots in FIG. 5(b) are presumed to be the Ag nanoparticles. This would indicate that the Ag nanoparticles supported in the pores are sparsely dispersed. The semi-conductive layer shown in FIGS. 5(a) and (b) includes the porous alumina layer **32A**. In other words, each pore **34A** in the porous alumina layer **32A** has a stepped side surface, and has two pore subportions with mutually differing pore diameters along the depth direction. In FIGS. 5(a) and (b), it is considered that the pore subportions at the deeper position produce darker images.

With reference to FIG. 7 and FIG. 8, a result of evaluating the lifetime of the electron emitting device of Example will be described. FIG. 7 schematically shows a measurement system for the electron emission characteristics of the electron emitting device **100**. FIG. 8 shows a result of an energization test (electron emission characteristics) for the electron emitting device **100** having the semi-conductive layer illustrated in FIGS. 5(a) and (b).

As shown in FIG. 7, on the second electrode **52** side of the electron emitting device **100**, a counter electrode **110** is disposed so as to oppose the second electrode **52**, and a current that occurs in the counter electrode **110** due to the electrons that are emitted from the electron emitting device **100** was measured. The following is assumed: a driving voltage **Vd** which is applied to the electron emitting device **100**; an intra-device current **Id**; a voltage **Ve** (which may be referred to as “collection voltage”) to be applied to the counter electrode **110**; and an emission current **Ie** occurring in the counter electrode **110**. The distance between the counter electrode **110** and the second electrode **52** was 0.5 mm, and the voltage **Ve** applied to the counter electrode **110** was 600 V. Herein, as shown in FIG. 7, the potential of the second electrode **52** was the ground potential, and a negative voltage was applied to the first electrode **12**. However, without being limited to this example, the potential of the second electrode **52** may only be higher than the potential of the first electrode **12** in order to allow electrons to be emitted from the second electrode **52**.

In FIG. 8, the intra-device current **Id**, the emission current **Ie**, and the emission efficiency **n** are plotted against energization time. The emission efficiency **η** is given as  $η = Ie/Id$ .

The emission efficiency **η** needs to be 0.01% or more, and may preferably be 0.05% or more.

The construction of the electron emitting device **100** produced is as follows.

5 first electrode **12**: a portion of JIS A1050 (thickness 0.5 mm) excluding any anodically oxidized portion

porous alumina layer **32A**: opening diameter **Dp** of about 100 nm, depth **Dd** of about 2200 nm, interpore distance **Dint** of 200 nm, porous alumina layer thickness **tp** of 2200 nm, barrier layer thickness **tb** of about 50 nm

10 deeper pore subportion: pore diameter **Dp1** of about 20 nm, depth **Dd1** of about 1500 nm

shallower pore subportion: pore diameter (opening diameter **Dp**) of about 100 nm, depth of about 700 nm

15 Ag nanoparticles **42n**: alcohol derivative-coated Ag nanoparticles contained in the aforementioned Ag nanoparticle dispersion, having an average particle size of 6 nm

second electrode **52**: Au layer (thickness 40 nm)

device size (size of the second electrode **52**): 5 mm×5 mm

20 The porous alumina layer **32A** shown in FIGS. 5(a) and (b) was formed by: performing an anodization with oxalic acid (0.05 M, 5° C.) and a formation voltage of 80 V for about 27 minutes; thereafter performing 20 minutes of etching with phosphoric acid (0.1 M, 25° C.); and thereafter 25 again performing an anodization with oxalic acid (0.05 M, 5° C.) and a formation voltage of 80 V for about 27 minutes.

25 After carrying out the aforementioned “forming” treatment, an energization test for the electron emitting device **100** was performed through an intermittent driving with ON 30 periods of 16 seconds and OFF periods of 4 seconds. The driving conditions are as follows. The driving voltage **Vd** (pulse voltage) applied between the first electrode **12** and the second electrode **52** was a rectangular wave having a frequency of 2 kHz and a duty ratio of 0.5, and the driving 35 voltage **Vd** was increased at a rate of 0.1 V/sec, until the emission current **Ie** reached a predefined value (which herein was  $4.8 \mu\text{A}/\text{cm}^2$ ) or greater. Thereafter, a feedback control of adjusting the driving voltage **Vd** was performed so that the emission current **Ie** as monitored with the counter electrode **110** 40 remained constant. The driving environment was 25° C., with a relative humidity RH of 30% to 40%.

As can be seen from FIG. 8, the electron emitting device **100** of Example had a lifetime of about 50 hours. Herein, lifetime of the electron emitting device is assumed to be the

45 length of time during which the emission current **Ie** maintained a certain value. Herein, assuming a usage as a charger device of a medium-fast copier machine, the length of time during which the emission current **Ie** maintained  $4.8 \mu\text{A}/\text{cm}^2$  was defined as the lifetime of the electron emitting device. 50 This value ( $4.8 \mu\text{A}/\text{cm}^2$ ) is estimated, given that the photo-sensitive drum of the medium-fast copier machine has a rotational speed of 285 mm/sec, to be an emission current that is needed to charge this photo-sensitive drum. As can be seen from FIG. 8, the emission current **Ie** of the electron emitting device **100** maintained  $4.8 \mu\text{A}/\text{cm}^2$  (i.e., a value indicated by a dotted line in FIG. 8) for about 50 hours.

55 From the study so far, it has been found that the lifetime can be made about 5 times longer (about 160 hours) by replacing the second electrode **74** (a single Au layer with a thickness of 40 nm) of an electron emitting device **200** of Comparative Example, which will be described later with reference to FIG. 9 (see Patent Document 2, for example), with a Pt layer/Au layer (20 nm/20 nm) layered structure. Therefore, by replacing the second electrode **52** of the electron emitting device **100** produced with the aforementioned layered structure, its lifetime will be prolonged to about 250 hours.

## 11

For comparison sake, a reference electron emitting device 200 was produced as shown in FIG. 9, and was similarly evaluated. FIG. 10 shows a result of an energization test (electron emission characteristics) for the electron emitting device 200 of Comparative Example. In FIG. 10, the intra-device current Id, the emission current Ie, and the emission efficiency  $\eta$  are plotted against energization time.

The construction of the electron emitting device produced is as follows.

first electrode 71: JIS A1050 (thickness: 0.5 mm)

dielectric layer 72: an anodic oxidized alumina layer (a porous alumina layer subjected to a sealing treatment), having a thickness of 4  $\mu$ m

semi-conductive layer 73: thickness of 1  $\mu$ m to 2  $\mu$ m

insulator 73m: silicone resin

Ag nanoparticles 73n: alcohol derivative-coated Ag nanoparticles contained in the aforementioned Ag nanoparticle dispersion, having an average particle size of 6 nm and accounting for 1.5 mass % with respect to silicone resin

second electrode 74: an Au layer (thickness 40 nm)

device size (size of the second electrode 74): 5 mm  $\times$  5 mm

The dielectric layer 72 was formed by a method similar to that of the dielectric layer 22 of the electron emitting device 100 described with reference to FIG. 2(a).

As can be seen from FIG. 10, the electron emitting device 200 produced as Comparative Example had a lifetime of about 50 hours. The lifetime of the electron emitting device 200 of Comparative Example was evaluated similarly to the electron emitting device 100 of Example.

FIG. 11 shows an example cross-sectional STEM image of the electron emitting device 200 of Comparative Example (not energized yet). FIG. 12 is a diagram showing a result of EDX analysis in a cross section of FIG. 11 (a region indicated with an open circle 2a in FIG. 11).

As can be seen from FIG. 11, Ag nanoparticles are present in regions indicated by circles in FIG. 11, for example. Within the silicone resin, a plurality of places where Ag nanoparticles are aggregated (e.g., inside the open circle 2a in FIG. 11) are created. The places where Ag nanoparticles are aggregated are nonuniformly distributed within the silicone resin.

Presumably, the distribution of Ag nanoparticles (including also a migration that may occur upon electric field application) may be somehow related to the electron emission characteristics and/or the device lifetime; however, no specific correlation has been established yet. However still,

## 12

Next, three kinds of electron emitting devices (test samples Nos. 1 to 3) as shown in Table 1 below were evaluated.

As illustrated herein, when the first electrode is formed by using a relatively rigid aluminum substrate (thickness 0.2 mm or more) containing aluminum with a purity of not less than 99.00 mass % and not more than 99.99 mass %, the aluminum substrate can be utilized as a support substrate, so that the electron emitting device can be efficiently produced.

Test samples Nos. 1 to 3 differ from one another with respect to the composition (e.g., aluminum content) of the aluminum substrate 12 used in forming the first electrode 12. The construction of test sample No. 1 (thickness: 0.5 mm) and the method of production it are basically identical with those of the electron emitting device 100 described with reference to FIG. 7 and FIG. 8. However, herein, the following steps were alternated to a total of three times each: a step of adding dropwise 200  $\mu$ L (microliter) of the aforementioned Ag nanoparticle dispersion onto the porous alumina layer 32A (a region which is about 5 mm  $\times$  about 5 mm); and a step of thereafter performing spincoating under conditions of 500 rpm for 5 seconds, and then 1500 rpm for 10 seconds. Thereafter, heating was performed at 150°C. for 1 hour. Test samples No. 2 (thickness: 0.5 mm) and No. 3 (thickness: 0.2 mm) were identical with test sample No. 1 except for the composition of the aluminum substrate 12.

Table 1 shows the main component in the composition of the respective aluminum substrate constituting the first electrode 12 of test samples Nos. 1 to 3.

Test sample No. 1 was produced by using JIS A1050 as the aluminum substrate 12. JIS A1050 has the following composition (mass %).

Si: 0.25% or less, Fe: 0.40% or less, Cu: 0.05% or less, Mn: 0.05% or less, Mg: 0.05% or less, Zn: 0.05% or less, V: 0.05% or less, Ti: 0.03% or less, others: each 0.03% or less, Al: 99.50% or more

Test sample No. 2 was produced by using JIS A1100 as the aluminum substrate 12. JIS A1100 has the following composition (mass %).

Si+Fe: 0.95% or less, Cu: 0.05% to 0.20%, Mn: 0.05% or less, Zn: 0.10% or less, others: each 0.05% or less and altogether 0.15% or less, Al: 99.00% or more

Test sample No. 3 was produced by using an aluminum base material containing aluminum in an amount of 99.98 mass % or more as the aluminum substrate 12. The aluminum substrate of test sample No. 3 had the following composition (mass %).

Si: 0.05% or less, Fe: 0.03% or less, Cu: 0.05% or less, Al: 99.98% or more

TABLE 1

| test  | composition (mass %) |                      |              |             |             |             |             |             |              |
|-------|----------------------|----------------------|--------------|-------------|-------------|-------------|-------------|-------------|--------------|
|       | sample               | Si                   | Fe           | Cu          | Mn          | Mg          | Zn          | Ti          | Al           |
| No. 1 |                      | $\leq 0.25$          | $\leq 0.40$  | $\leq 0.05$ | $\leq 0.05$ | $\leq 0.05$ | $\leq 0.05$ | $\leq 0.03$ | $\geq 99.50$ |
| No. 2 |                      | Si + Fe: $\leq 0.95$ | 0.05 to 0.20 | $\leq 0.05$ | —           | $\leq 0.10$ | —           | —           | $\geq 99.00$ |
| No. 3 |                      | $\leq 0.05$          | $\leq 0.03$  | $\leq 0.05$ | —           | —           | —           | —           | $\geq 99.98$ |

the electron emitting device according to an embodiment of the present invention allows Ag nanoparticles to be supported in the pores of the porous alumina layer, and the Ag nanoparticle distribution can be controlled by controlling the opening diameter, depth, interpore distance, etc., of the pores. Therefore, the characteristics of the electron emitting device can be improved and/or a long lifetime can be achieved.

The energization test for test samples Nos. 1 to 3 was performed basically similarly to the energization test described with reference to FIG. 8. However, for simplicity's sake, no feedback control for the driving voltage Vd was performed. Specifically, after performing the aforementioned "forming" treatment, the driving voltage Vd (a rectangular wave having a frequency of 2 kHz and a duty ratio of 0.5) was increased to 26 V at a rate of 0.05 V per cycle,

and thereafter maintained at 26 V. Note that one cycle of intermittent driving consists of an ON period of 16 seconds and an OFF period of 4 seconds. The driving environment was 20 to 25° C., with a relative humidity RH of 30% to 40%.

In any of test samples Nos. 1 to 3, when the driving voltage  $V_d$  was about 10 V or more, the emission current  $I_e$  gradually increased. By confirming that the emission current  $I_e$  increased with an increasing driving voltage  $V_d$ , it was determined that it was operating as an electron emitting device. Thus, it was confirmed that each of test samples Nos. 1 to 3 was operating as an electron emitting device.

Table 2 shows results of determining an average value of emission current  $I_e$  for each test sample. In Table 2, “Δ” indicates that an average value of emission current  $I_e$  was not less than 0.001  $\mu\text{A}/\text{cm}^2$  but less than 0.01  $\mu\text{A}/\text{cm}^2$ ; “○” indicates that an average value of emission current  $I_e$  was not less than 0.01  $\mu\text{A}/\text{cm}^2$  but less than 0.1  $\mu\text{A}/\text{cm}^2$ ; and “◎” indicates that an average value of emission current  $I_e$  was not less than 0.1  $\mu\text{A}/\text{cm}^2$  but less than 4.8  $\mu\text{A}/\text{cm}^2$ .

TABLE 2

|                                         | test sample |       |       |
|-----------------------------------------|-------------|-------|-------|
|                                         | No. 1       | No. 2 | No. 3 |
| average value of emission current $I_e$ | ○           | ◎     | Δ     |

Test sample No. 2, in which the purity (i.e., ratio of aluminum content of the aluminum substrate) was lower than that of test sample No. 1, had an average value of emission current  $I_e$  which was greater than that of test sample No. 1. On the other hand, test sample No. 3, in which the purity (ratio of aluminum content) of the aluminum substrate was higher than that of test sample No. 1, had an average value of emission current  $I_e$  which was smaller than that of test sample No. 1. Thus, as the purity (ratio of aluminum content) of the aluminum substrate decreased, the average value of emission current  $I_e$  increased.

However, the aforementioned energization test only illustrates exemplary driving conditions. Depending on the driving conditions of the electron emitting device, the value of emission current  $I_e$  may vary. Under operation with a large average value of emission current  $I_e$  (i.e., amount of electron emission per unit time), the duration in which operation as an electron emitting device is possible may decrease. As used herein, “the duration in which operation as an electron emitting device is possible” means the period from the moment at which operation as an electron emitting device is confirmed to the moment at which the value of emission current  $I_e$  decreases for the same driving voltage  $V_d$ ; note that this definition differs from that of “lifetime” (i.e., the length of time during which the emission current  $I_e$  maintained a certain value) which was described with reference to FIG. 8, for example.

The value of emission current and the duration of operation that is expected of an electron emitting device may vary depending on the application (i.e., driving conditions). However, in applications where large emission current values are required, for example, it is preferable to use an aluminum base material with a relatively low aluminum purity (not less than 99.00 mass % and not more than 99.50 mass %). In applications where long hours of operation is highly regarded, for example, it is preferable to use an aluminum base material having a relatively high aluminum purity (not less than 99.50 mass % and not more than 99.98 mass %).

The exact mechanism by which the aluminum purity affects the characteristics of the electron emitting device is not clear as yet. However, as seen from Table 1, any element that is contained as an impurity in the aluminum substrate used herein, except for Mg, is an element which has a high standard electrode potential (i.e., so-called “noble”) as compared to aluminum. Therefore, an impurity element(s) (e.g., iron) that is more noble than aluminum may possibly be affecting the characteristics of the electron emitting device.

## INDUSTRIAL APPLICABILITY

Embodiments of the present invention may be suitable as an electron emitting device for use in a charger device of an image forming apparatus, or a method of producing the same, for example.

## REFERENCE SIGNS LIST

- 20 12: first electrode (aluminum substrate)
- 22: dielectric layer
- 30, 30A: semi-conductive layer
- 32, 32A, 32B, 32C: porous alumina layer
- 32b: barrier layer
- 34, 34A, 34B, 34C: pore
- 42: silver (Ag) supported in pores 34
- 42n: Ag nanoparticle
- 52: second electrode
- 71: first electrode
- 72: dielectric layer
- 73: semi-conductive layer
- 73m: insulator
- 73n: Ag nanoparticle
- 74: second electrode
- 100, 200: electron emitting device

The invention claimed is:

1. An electron emitting device comprising a first electrode, a second electrode, and a semi-conductive layer provided between the first electrode and the second electrode, wherein

the semi-conductive layer includes a porous alumina layer having a plurality of pores and silver supported in the plurality of pores of the porous alumina layer, and the first electrode is formed of an aluminum substrate containing aluminum in an amount of not less than 99.00 mass % but less than 99.99 mass %, and the porous alumina layer is an anodized layer formed at a surface of the aluminum substrate.

2. The electron emitting device of claim 1, wherein the first electrode is formed of an aluminum substrate or an aluminum layer, and the porous alumina layer is an anodized layer formed at a surface of the aluminum substrate or at a surface of the aluminum layer.

3. The electron emitting device of claim 1, wherein aluminum is contained in an amount of 99.98 mass % or less in the aluminum substrate.

4. The electron emitting device of claim 1, wherein the porous alumina layer has a thickness which is not less than 10 nm and not more than 5  $\mu\text{m}$ .

5. The electron emitting device of claim 1, wherein the plurality of pores have an opening having a two-dimensional size which is not less than 50 nm and not more than 3  $\mu\text{m}$  as viewed from a normal direction of a surface thereof.

6. The electron emitting device of claim 1, wherein the plurality of pores of the porous alumina layer have a depth which is not less than 10 nm and not more than 5  $\mu\text{m}$ .

**15**

7. The electron emitting device of claim 1, wherein a barrier layer included in the porous alumina layer has a thickness which is not less than 1 nm and not more than 1  $\mu\text{m}$ .

8. The electron emitting device of claim 1, wherein the second electrode includes a gold layer.

9. An electron emitting device comprising a first electrode, a second electrode, and a semi-conductive layer provided between the first electrode and the second electrode, wherein

the semi-conductive layer includes a porous alumina layer having a plurality of pores and silver supported in the plurality of pores of the porous alumina layer, and the plurality of pores of the porous alumina layer have a stepped side surface.

10. An electron emitting device comprising a first electrode, a second electrode, and a semi-conductive layer provided between the first electrode and the second electrode, wherein

the semi-conductive layer includes a porous alumina layer having a plurality of pores and silver supported in the plurality of pores of the porous alumina layer, and the silver contains silver nanoparticles having an average particle size which is not less than 1 nm and not more than 50 nm.

**16**

11. A method of producing an electron emitting device comprising a first electrode, a second electrode, and a semi-conductive layer provided between the first electrode and the second electrode, wherein

the semi-conductive layer includes a porous alumina layer having a plurality of pores and silver supported in the plurality of pores of the porous alumina layer, the method comprising:

a step of providing an aluminum substrate or an aluminum layer supported by a substrate;

a step of anodizing a surface of the aluminum substrate or the aluminum layer to form a porous alumina layer; and

a step of applying silver nanoparticles in a plurality of pores of the porous alumina layer.

12. The production method of claim 11, wherein the step of forming the porous alumina layer comprises an anodization step and an etching step to be performed after the anodization step.

13. The production method of claim 12, wherein the step of forming the porous alumina layer comprises a further anodization step after the etching step.

\* \* \* \* \*